

## UNITED STATES PATENT OFFICE

2,149,282

## MANUFACTURE OF PAINT

Emile C. De Stubner, Charleston, W. Va.

No Drawing. Original application December 28, 1935, Serial No. 56,585. Divided and this application May 7, 1937, Serial No. 141,241

5 Claims. (Cl. 134—39)

The present application is a division of my pending application Serial No. 56,585, entitled "Method and process of converting non-aqueous pulps."

The present invention relates to a process for incorporating finely divided solids into vehicles which may form a part of ultimate consumer products. The process achieves a fine subdivision of the finely divided solids and their substantially uniform and complete dispersion into the vehicle, while eliminating the customary grinding of such solids into the vehicle.

Finely divided solids dispersed in a dispersion medium to form a pulp have an individual particle size and a completeness of dispersion which is very desirable to maintain in the consumer product. The dispersion mediums which act best as pulping mediums for finely divided solids are mobile liquids. The formation of pulps of finely divided solids dispersed in a mobile pulping medium of an aqueous liquid has heretofore been suggested. The use of such aqueous pulps and their incorporation directly into the commonly utilized vehicles has not been satisfactory because such vehicles usually are less mobile than such pulping mediums and are immiscible therewith. The presence of the aqueous liquid in the pulp thus tends to impair the quality and completeness of the dispersion and is not practical from the commercial standpoint because of the difficulties inherent in removing the water from the completed dispersion. I have found that mobile liquids of a non-aqueous nature may be used in forming the initial pulp. Such pulps may be formed from pulps in which the pulping medium is an aqueous liquid or the solid particles may be pulped directly into the non-aqueous mobile liquid as the pulping medium.

In the present process, therefore, I propose to utilize the desirable properties of the pulp form of finely divided solids in a mobile non-aqueous pulping medium which is relatively more volatile than the vehicle into which the solids are to be incorporated in the process. By so doing it is possible to secure dispersion of the finely divided solids directly into the vehicle without grinding the solids in the vehicle. The pulping mediums which may be used satisfactorily in the present process are chiefly mobile liquids of a non-aqueous nature which are miscible in or compatible with the selected final dispersion mediums and are relatively more volatile than such dispersion mediums. In each instance such pulping medium should be selected which has a surface tension lower than the surface tension of the final dis-

persion medium and one which has a preferential affinity for the finely divided solid particles, so that the pulping medium acts as an efficient wetting agent for the finely divided solids. Among such pulping mediums are liquids in the field of organic solvents, such, for example, as toluene, benzene, acetone, turpentine, and the like. The use of such pulping medium will be found to preserve the beneficial features of the pulp formed of finely divided solids in a mobile pulping medium in such a manner as actually to facilitate the transfer of the finely divided solids to the final dispersion medium which may be the vehicle of a consumer product.

Thus one of the objects of the present invention is to utilize the non-aqueous pulp form of finely divided solids in the art of compounding. It is well known that finely divided solids are now combined in a direct manner with other elements in which combination these finely divided solids are the necessary and desired constituents. A great number of various types of mechanical devices are employed by chemical manufacturers in the preparation of such combinations, and it is my purpose to disclose a process and method whereby these finely divided solids in pulp form may be more readily and advantageously combined with such products, in order thereby to simplify such processes, while at the same time producing superior products inasmuch as these finely divided solids will be more uniformly distributed in such products by the present process than by previously known processes.

It is a further object of the present invention to provide a method for converting non-aqueous pulps of finely divided solids and to displace or replace either wholly or partially the non-aqueous pulping medium of such pulps by other constituents or vehicles of the desired product. In other words, to disclose a process adapted to the incorporation of finely divided solids such as abrasives, fillers, colors, and the like, into products useful as and/or in the manufacture of adhesives, insecticides, leather, leather finishes, artificial leather, printing ink, soap, candles, cosmetics, lubricants, rubber goods, tires, paint, paint enamels, matt varnishes, varnish stains, oil stains, putty, wood finishes, metal finishes, flattening compounds, polishes, floor wax, sealing wax, coating compositions, thermoplastics, molding compounds, plastics, Celluloid, lacquer, oilcloth, linoleum, etc.

In a preferred embodiment of the present invention, a further object is to disclose a method of replacing the volatile pulping medium of the finely divided solids in pulp form in its vapor

phase under atmospheric pressure, increased pressure, or diminished pressure (vacuum), by a non-volatile constituent, the latter constituent being a component also of the final and/or consumer product. Such preferred embodiment consists in general in the transformation of the solids of non-aqueous pulps having a volatile pulping medium into non-volatile constituents, vehicles, or composites.

10 Further and additional objects of the present invention will more readily appear in the perusal of my specification and examples.

While the present process possesses economical advantages over present methods, the product made in accordance with my teachings is of excellent quality and derives a distinctive and pleasing appearance and/or superior effectiveness from the uniformity and evenness of size and dispersion of the finely divided solids, whether 15 abrasive, color or filler, from the nature and characteristics of the parent pulps having a non-aqueous volatile pulping medium. This mark of uniformity of appearance and superior effectiveness which distinguishes the individual batch or run may be found in any number of successive 20 batches or runs. Thus variations of or in manufacture may be substantially eliminated by the present process which excludes to a large extent the human element and substitutes therefor a 25 control of the process based on the physical constants of the volatile pulping medium as well as the relatively non-volatile replacing or displacing 30 constituents.

The quality of the above-enumerated products 35 depends largely upon the fineness of their incorporated solids and to a even greater extent upon their even distribution in their vehicles. It is technically far easier to obtain pulps of these solids when the pulping medium is a volatile mobile liquid in which the solids possess a high degree of fineness, than in an oil or heavy viscous 40 or plastic vehicle. Therefore, I have selected and desire to employ these solids in their pulp form, preferably utilizing non-aqueous pulping mediums 45 of a relatively volatile nature. This is distinguishable over present manufacturing methods which utilize the finely divided particles in the dry state. I have discovered that such a pulping medium may be displaced or replaced by a non-volatile vehicle incorporating the solid constituents 50 of such pulps by applying this principle of replacement or displacement in my novel process to obtain a most even and uniform distribution of said solids into the vehicle.

55 A further object which will appear clearly from my specification and examples is to disclose, as one method, whereby this displacement or replacement of the non-aqueous volatile pulping medium by a non-volatile constituent of the product 60 may be accomplished, a distillation method under atmospheric pressures or vacuum and/or increased pressures, either with or without the use of agitation and in the presence of non-volatile replacing or displacing constituents or vehicles.

70 For the purpose of clarifying the terms used herein, I hereby define "pulps" as being any soft or semi-liquid mixtures of solid particles in liquids, the liquids being hereinafter referred to as the pulping mediums.

75 By the use of the term "non-aqueous" I intend to include substances chiefly of an organic nature which are substantially free of water or aqueous liquids and by the use of such term to

exclude the substances which are chiefly of water or of an aqueous nature.

The term "dispersion medium" as used herein includes substances forming a component element of the end or consumer product and which may exist either as a liquid or a plastic under the conditions existing at the time of the volatilization of the non-aqueous pulping medium. Such dispersion medium may exist under normal atmospheric temperatures and pressures, either as a solid or plastic such as a resin, or as a liquid such as an oil.

In order that the present invention may be more clearly understood and the process of converting pulps of finely divided solids having a non-aqueous volatile pulping medium into compounds having non-volatile constituents, it is essential that the non-volatile constituent must displace or replace the volatile pulping medium and that this must be accomplished at the same time that the finely divided solids are uniformly distributed throughout the non-volatile constituent or produce. Any method whereby the non-volatile constituent or vehicle or product is caused to replace or displace the non-aqueous volatile pulping medium falls within the scope of the present invention and claims, but in a preferred embodiment thereof I employ distillation and in some cases distillation and agitation. I may so control this conversion that as the volatile pulping medium is driven off, the non-volatile constituent replaces the same in such manner as to assure that the finely divided solid is evenly and uniformly distributed into the non-volatile constituent or vehicle.

The following examples are illustrative of the operation of my invention and processes and are here included for such purpose and not for the purpose of limitation.

#### Example I

In order to make "Prussian Blue in Oil" I proceed as follows: 100 lbs. of toluene Prussian blue pulp of 30% pigment content is mixed with 30 lbs. of linseed oil. This mixture is then subjected to distillation and agitation until the 70 lbs. of toluene of the Prussian blue pulp are distilled off.

In practice I prefer to employ a kneading machine of the type of Werner & Pfleiderer or other suitable type which is provided with a jacket, hollow agitating blades, a tight cover, a still neck, an attached condenser, an inlet valve which permits feeding for continuous operation, and thermometer wells for measuring the temperatures of the machine contents as well as the vapor in the still neck. In such an apparatus distillation may proceed under atmospheric pressures or under either increased or diminished pressures. Into such apparatus I place 1000 lbs. of Prussian blue toluene pulp of 30% pigment content and 300 lbs. linseed oil. The blades revolve at a speed of 60 R. P. M. The cover is tightly closed and connected with the still neck and condenser which in turn are tightly connected with a 300-gallon receiver and the latter joined with a vacuum creating source. The temperature of the mix is now raised to 75° C. by means of suitable means either in the jacket or in the hollow blades. While this batch is agitated by the blades which exert a smearing or kneading or squeezing action, the vacuum line is opened and a vacuum of 25 to 27 inches of mercury is created inside the apparatus. Under these conditions the toluene is distilled off and there remains in the apparatus 60 lbs. of "Prussian Blue in Oil" (in this case linseed

oil) which may be discharged through a valve in the bottom or by tilting or any other convenient means.

*Example II*

For making "Chrome Orange in Japan", I place in the apparatus of Example I, 1000 lbs. of 50% basic lead chromate acetone pulp and 500 lbs. of "Grinding Japan" and distill off the acetone.

I may in a similar way, proceed to convert the 10 fillers or pigments or abrasives necessary in the production of any of the products outlined above or other similar consumer products or intermediate products.

In the foregoing examples of processes embodying the present invention, it will be noted that in each instance a pulp of the finely divided solids in a non-aqueous pulping medium, which is relatively more volatile than the dispersion medium, is admixed with the dispersion medium and is then volatilized and dissociated from the mixture, whereupon the finely divided solids are transferred to and suspended in the dispersion medium. In each instance the pulping medium is compatible with or miscible in the dispersion medium prior to its volatilization and removal from the admixture.

By the term "Grinding Japan" as used herein is meant a varnish of the type commonly used in "Japanning" of metal or wooden articles and which is also used as a vehicle into which pigments may be ground by conventional grinding processes.

While I have named particular substances for particular purposes in the foregoing examples, I 35 do not wish to be limited thereby to the utilization of such substances or such purposes as the present process is adaptable to many other purposes, using many substances other than those particularly specified.

40 I claim:

1. The process of manufacturing paint which includes the steps of providing a suitable quantity of a substantially water-free finely divided pigment pulped in a substantially water-free volatile thinner for the paint vehicle and which has a greater wetting action on the pigment than does the said vehicle, admixing a suitable portion of a selected non-volatile paint vehicle therewith, placing the admixed pigment, thinner and 45 vehicle in a still, subjecting said admixture in the still to simultaneous heating and kneading to distill off a predetermined amount of said thinner while retaining the pigment particles in finely

divided condition and substantially uniformly dispersed in the mass, whereby the excess thinner is removed and the admixture is concentrated with the pigment particles dispersed in said vehicle and any remaining thinner.

2. The process of manufacturing a blue colored paint which comprises admixing a substantially water-free toluene pulp of Prussian blue pigment with linseed oil, thereafter simultaneously kneading the mixture and distilling off a predetermined amount of the toluene while maintaining the pigment particles in a dispersed condition, whereby the consistency of the composition is increased and the Prussian blue pigment is dispersed in the linseed oil and any remaining toluene as the vehicle of the coating composition.

3. The process of manufacturing an orange colored paint which comprises admixing a substantially water-free acetone pulp of basic lead chromate with "Grinding Japan", and thereafter simultaneously kneading the mixture and distilling off predetermined amounts of the acetone while maintaining the pigment particles in a dispersed condition, whereby the consistency of the composition is increased and the basic lead chromate is dispersed into the said "Grinding Japan" and any remaining acetone as the vehicle of the coating composition.

4. A method of incorporating pigment into a paint vehicle by kneading the mass, which comprises admixing the pigment, a substantially water-free volatile wetting agent therefor, and a substantially water-free paint vehicle miscible with the said wetting agent, to form a mixture in which the pigment is thoroughly wetted by the 30 agent and vehicle, thereafter distilling off a desired amount of the wetting agent and kneading the mass simultaneously during said distillation, whereby the consistency of the mass is increased 35 and the pigment is uniformly dispersed in the vehicle and any remaining wetting agent.

5. The process of bodying a paint mixture and improving the quality of dispersion of pigment therein which consists in subjecting a paint mixture consisting of pigment, a substantially water-free non-volatile vehicle and a substantially water-free volatile thinner to a simultaneous kneading and distillation, whereby a predetermined amount of the said thinner is removed and the dispersion of the pigment particles in the remaining vehicle and thinner is improved while the bulk of the original paint mixture is reduced.

EMILE C. DE STUBNER.